

Sept. 24, 1935.

C. S. PRICE

2,015,605

METAL SEAL AND PROCESS OF MAKING

Original Filed Sept. 24, 1928



Fig. 1



Fig. 2



Fig. 3



Fig. 4



Fig. 5



Fig. 6



Fig. 7

WITNESS

Edwin L. Bradford

INVENTOR:  
Chas. S. Price

BY

Towson Price  
ATTORNEY

## UNITED STATES PATENT OFFICE

2,015,605

## METAL SEAL AND PROCESS OF MAKING

Charles S. Price, Hollis, N. Y.

Application September 24, 1928, Serial No. 307,990  
Renewed September 13, 1933

14 Claims. (Cl. 154—2)

This invention relates to metal seals, labels, letters and the like and the method of making the same where it is desired that such articles may be quickly and easily affixed to paper, card-board, leather, cloth and the like.

The principal object of my invention, generally considered, is to improve on the process of making metallic characters or seals with adhesive on the backs thereof which is adapted for 10 remoistening whereby said adhesive will not chip off the metal but will act to effectively hold the seal or other character to any desired article.

Another object of my invention is to provide such a metal seal provided with a thin coating 15 of adhesive possessing all the qualities necessary in a successful article of this kind and at the same time produce cheaper seals by reason of a simplified procedure.

A further object is to provide a seal of this 20 character provided with an adhesive backing relatively thin as compared with the backing previously used and which, by reason of its thinness, is more flexible, lending itself more readily to delicate embossing and conforming 25 more closely to the surface to which it is attached.

A still further object of my invention is to produce a metal seal, label or the like provided with 30 a coating of adhesive on the back, such coating being strongly adherent to the metal seal and also to any surface to which it may be attached after remoistening so that it will strongly resist any attempts to remove it after attachment, having no distinctly separate layers as in the case of 35 such articles previously produced, being homogeneous, although composite layers of adhesives and not a combination of dissimilar substances.

Other objects and advantages of the invention relating to the particular arrangement and construction of the various parts will become apparent as the description proceeds.

Metal seals with glue or other adhesive on the backs have previously been made in a complicated manner, due to the fact that it has been 45 impossible to obtain a suitable adhesive which can be remoistened and which at the same time had sufficient adhesion to the metal portion of the seal and to the article to which it was desired that it should be affixed. There appeared to be 50 no adhesive which possessed all the requisites for this purpose, namely, ability to be easily remoistened; quickly adhesive to any substance; permanently adherent to the metal seal; flexible after drying to permit forming, embossing and 55 shearing operations on the metal after coating;

not corrosive or deliquescent; and, lastly, having a not unpleasant odor or taste.

In accordance with my process, a strip of metal is preferably first cleaned on both sides, either by passing it through a chemical cleaner or 5 subjecting it to mechanical brushing, or both. The side to which it is desired to apply the adhesive is then passed in contact with a revolving roll of a coating machine and supplied with the first coating of adhesive. This consists of 10 an adhesive such as a good pyroxylin lacquer, or a high grade linseed oil varnish, which has a strong adhesive action with respect to metal but which is not capable of being remoistened. This first coat of adhesive is permitted to dry and a 15 second coat of a different adhesive, capable of being remoistened, is applied thereto. This second coat is then allowed to become dry and the metal is then ready for manufacture into seals, 20 labels or the like by any one of the several methods known to those skilled in the art.

As an alternative, however, I may apply to the metal, after the application of the first adhesive or varnish, an intermediate paper or fibrous strip and subsequently apply to the other side of said 25 strip the glue or other adhesive capable of being remoistened. The second coating of remoistening adhesive would not, if used by itself, have sufficient adhesion to the metal but it does 30 exhibit strong adhesion to the first layer of adhesive or to the intermediate paper backing so that I am actually accomplishing with the combined coating of two different adhesives a result different from anything heretofore known 35 in the art.

Referring to the drawing illustrating my invention, the scope whereof is defined by the appended claims.

Figure 1 shows apparatus embodying my invention for treating strips of metal and paper or 40 other fibrous material with adhesive, rolling them into intimate contact, baking and applying the remoistening adhesive to the baked paper backed metal.

Figure 2 shows a modified apparatus for performing a slightly different process.

Figure 3 shows a further modified apparatus for performing a still further modified process in accordance with my invention.

Figure 4 is a front elevation of a metal seal produced in accordance with my invention.

Figure 5 is a cross sectional view of such a seal.

Figure 6 is a front elevation of another form 55

of seal produced in accordance with my invention.

Figure 7 is a cross sectional view of such a seal.

Referring to the drawing in detail, like parts being designated by like reference characters, and first considering the embodiment of my invention illustrated in Figure 1, I show a roll of metal tape 1, a strip of metal 2 from which is drawn preferably first over an idler pulley 3 and across a cement, varnish or other adhesive applying roll 4. It will be noted that the roller 4 dips into a tank 5, which may contain a good pyroxylin lacquer or high grade linseed oil varnish, although it should be understood that I am not limited to using such an adhesive, as, if desired, I might use a water soluble glue in general designated as not remoistening, such as glue being soluble with difficulty when heated, such as wood glue, or other adhesive.

After having the first coat applied by the roller 4 the metal tape may pass over another idler pulley or roller 6 and into a drying oven 7, being supported in said oven by rods or rollers 8, wherein it is thoroughly dried. After emerging from the oven 8 it may pass over a series of idler pulleys or rollers 9, 10, 11, and 12 and finally over an adhesive applying roller 13, where it receives the second or final coat of adhesive, such latter adhesive being remoistening liquid glue or the like.

After having the final coating of adhesive applied, the strip of metal preferably passes over another idler pulley 14 and through another drying oven 15, being held in position as heretofore by rods or rollers 16 therein, where it is thoroughly dried and subsequently preferably rolled up on the final roll 17 by means of a motor or other source of power 18.

In the foregoing description I have not referred to the roll of paper 19 which may be combined with the metal strip after application of the first adhesive thereto, but it will be understood that, if desired, after the first adhesive has been applied by the roller 4, the strip of paper 20 from the roll 19 may be combined with the strip of metal 2 by being rolled into intimate contact therewith by passing through the rollers 21 adjustably pressed together, as by means of set screws 22. After the paper and metal have been thus firmly pressed together, the composite strip passes through the drying oven 7, as heretofore described, where it is thoroughly dried and afterwards the paper backed side of the strip has the second or remoistening adhesive applied thereto by the roller or drum 13 which dips into the tank of water soluble remoistening adhesive 23. After having the second coating of adhesive applied thereto the composite strip is then dried in a second oven 15 and reeled upon the roller 17.

Referring now to the embodiment of my invention illustrated in Figure 2, a form of apparatus is illustrated in which a roll of metal tape 1<sup>a</sup> supplies a strip of metal 2<sup>a</sup> which is drawn over an adhesive applying roller 4<sup>a</sup> which is kept supplied with varnish, lacquer or the like by dipping into a tank 5<sup>a</sup> thereof, the lower side of said metal being coated with the primary adhesive simultaneously with the application of lacquer or the like to the other side of said metal, as by means of a spray 24. The purpose of applying the lacquer to the other side of the metal is to protect it against tarnish and act as a size when the labels are later printed. The first coat of adhesive is preferably given a preliminary

drying in the oven 7<sup>a</sup> and while still tacky rolled by means of rollers 21<sup>a</sup>, into intimate contact with a paper intermediate layer 20<sup>a</sup> drawn from a roll 19<sup>a</sup>. The composite strip of metal and paper is finally dried or baked, preferably in an oven 15<sup>a</sup>, and reeled upon the roll 7<sup>a</sup>, as in the previous embodiment. It will be noted that in the present embodiment the application of the second coat of adhesive has not been described. Such temporary omission of the final adhesive may, in some cases, be advisable as it permits storing the metal without the final water soluble gum which sometimes causes trouble due to deterioration when stored for a long time. Such incompletely prepared strip can be coated with the final gum on the paper backing just as it is needed.

Referring now to the embodiment of my invention illustrated in Figure 3, an apparatus is there disclosed in which the preliminary coating of adhesive is sprayed on the metal by means of a sprayer 4<sup>b</sup>, the strip of metal 2<sup>b</sup> being drawn from a roll 1<sup>b</sup> passed through a drying oven 7<sup>b</sup> and while still tacky rolled into intimate contact with a strip of paper 20<sup>b</sup> drawn from a roller 21<sup>b</sup>, said metal and paper passing through pressure rollers 21<sup>b</sup> and then through a drying oven 15<sup>b</sup> and rolled on a roller 17<sup>b</sup>. It will be understood that the apparatus illustrated in both Figures 2 and 3 may be supplemented by an adhesive coating roller and tank, such as illustrated in Figure 1 at 13 and 23, so that the composite strip may be immediately coated with the final glue and then dried in an oven, such as shown at 15, before being reeled and stored. 3

Referring now to the seal illustrated in Figures 4 and 5, there is here shown the final product resulting from my process and manufactured by the apparatus heretofore described, that is, it will be understood that after the strip 4 of metal, which is preferably heavier than foil so as to hold its shape after forming, is coated and dried, as desired, it is printed or decorated, stamped or embossed and cut to form seals or the like of any desired character. Figures 4 and 5 illustrate a seal with the number 1 embossed thereon, the metallic outer or front portion 25 of which has a preliminary backing 26 of one adhesive and a second coat 27 of a different adhesive. The first adhesive, preferably waterproof, acts as a binder between the remoistening glue or second adhesive 27 and the metal to permit it being formed, embossed and cut without chipping or peeling. 5

Figures 6 and 7 show another product of my process wherein is produced a seal with a metal outer or front layer 25<sup>b</sup> having a preliminary coating of a preferably waterproof adhesive 26<sup>b</sup>, say varnish or lacquer, then a thin layer of paper 28, and finally a coat of remoistening gum 27<sup>b</sup>. 6 The function of the paper is to accelerate the rate of setting of the remoistening gum by providing a capillary passageway for the moisture to the edge of the seal when the seal is attached to a non-absorptive surface, such as 6 glass. 7

From the foregoing it will be seen that I have provided a method and apparatus for producing metal seals in which two different adhesives are used, with or without a paper or fibrous layer 7 therebetween; whereby the metal portion, which is desirably formed of brass or other non-rusting metal, is adapted to be firmly held upon any article to which it is applied. It will also be understood that the term "varnish" is used in its broad 7

sense, as a material which serves as an adhesive and gives a varnish-like or waterproof coating.

Having thus described my invention, I claim:

1. The process of making metal characters and the like for attachment to various materials comprising coating a metal strip with an oil varnish, drying said coat, applying liquid glue to the varnish coat, drying the glue, forming characters on the metal, and severing said characters one from the other.

2. The process of making metal characters and the like for attachment to various materials comprising coating a metal strip with varnish, drying said coat, applying liquid glue to the varnish coat, drying the glue, forming characters on the metal, and severing said characters one from the other.

3. In the process of making metal characters that will strongly adhere to various materials, the steps which comprise coating a metal strip with varnish, drying said coat, and applying liquid glue to the varnish coat.

4. A metal seal comprising a layer of metal, a coating of an oil varnish, and a coating of remoistening glue on said varnish, said seal being ornamented on the other side of the metal.

5. A metal seal comprising a layer of metal, a coating of varnish, and a coating of remoistening glue on said varnish, said seal being ornamented on the other side of the metal.

6. The process of making metal characters and the like for attachment to various materials, comprising coating a metal strip with varnish, drying said coat, applying liquid glue to the strip on the same side as the varnish, drying the glue, forming characters on the metal, and severing said characters one from the other.

7. In the process of making metal characters that will strongly adhere to various materials, the steps which comprise coating a metal strip with varnish, drying said coat, and applying liquid glue to the strip on the same side as the varnish coat.

8. A metal seal comprising a layer of metal, a first coating of varnish, and a coating of remoistening glue on the seal and secured to the varnish,

said seal being ornamented on the other side of the metal.

9. The process of making metal characters and the like for attachment to various materials, comprising coating a metal strip with a waterproof adhesive, attaching a strip of paper to said metal strip by means of said adhesive, drying the composite strip, applying liquid glue to the paper of said strip, drying the glue, forming characters on the composite strip, and severing said characters one from the other.

10. In the process of making metal characters that will strongly adhere to various materials, the steps which comprise coating a metal strip with a waterproof adhesive, attaching a strip of paper thereto by means of said adhesive, drying the composite strip, and applying liquid glue to the paper coated side of said strip.

11. A metal seal comprising a layer of a coating of a waterproof adhesive, a layer of paper attached to said metal by means of said adhesive, and a coating of remoistening glue on the outer surface of the paper, said seal being ornamented on the other side of the metal.

12. The process of making metal characters and the like for attachment to various materials, comprising coating a metal strip with a waterproof adhesive, drying said coating, applying liquid glue to the strip on the same side as the waterproof adhesive, drying the glue, forming characters on the metal, and severing said characters one from the other.

13. In the process of making metal characters that will strongly adhere to various materials, the steps which comprise coating a metal strip with a waterproof adhesive, drying said coating, and applying liquid glue to the strip on the same side as the waterproof adhesive.

14. A seal comprising a layer of metal, a first coating of a waterproof adhesive, and a coating of remoistening glue on the seal and secured to the waterproof adhesive, said seal being ornamented on the other side of the metal.

CHARLES S. PRICE.